

## UNITED STATES PATENT OFFICE

2,187,858

## METHOD OF PRODUCING IMPREGNATING COMPOSITIONS

Rudolf Kern, Oschatz, Germany, assignor to the firm Chemische Fabrik R. Baumheier Kommanditgesellschaft, Oschatz-Zschöllau, Germany

No Drawing. Application April 15, 1936, Serial No. 74,593. In Germany August 6, 1936

3 Claims. (Cl. 134—15)

My invention relates to improvements in dispersed substances and the process for making such substances as well as the fabrics to the fibres of which the substance is absorbed.

5 It has heretofore been proposed to render fabrics water-proof by impregnating the same with soaps of multivalent metals. Ordinarily the fabric is first placed in a bath of alumina and then in a soap bath, or vice versa. In this connection the soap bath, which has no water-proofing effect in itself, may also contain water-insoluble substances, such as wax, paraffin, or the like. In this process, therefore, two or more baths are required. In another process the fabrics are 10 treated in a preformed organic solution of aluminum soaps in solvents. This process, however, is expensive and uneconomical owing to the loss of solvent. To avoid these disadvantages it has also been proposed to treat the fabric in aqueous 15 suspensions of aluminum soaps formed merely by a simple stirring process. This method, however, has not only the disadvantage of instability of the liquors but also that of irregularity of the impregnation. Since in the ordinary way of 20 production the aluminum soaps occur in the form of comparatively large particles, the impregnation is irregular, and these comparatively large structures are unable to penetrate the fabric. For this reason the impregnation is unsatisfactory. The aluminum soaps adhere to the 25 fabric merely superficially and are easily rendered ineffective when the fabric is in use. There is also obtained an inferior finish, and the fabric is coarse to the touch.

25 The object of the present improvements is to provide a process which is free of the said objections, and with this object in view my invention consists in manufacturing emulsions which are capable of resisting storage, transport and frost and are simple and economical to handle. In the following there will be described the composition of the emulsion, its production, and the manner in which the process is employed.

1. The emulsions consist of soaps of multivalent metals, and more particularly of aluminum, magnesium, zinc, lead or copper. The acid radicals of these soaps of multivalent metals are formed from saturated or unsaturated fatty acids, waxy acids, resin acids or naphthene acids. 30 Fatty acids are understood to be those which result in soaps by dissolution with alkalis. These fatty acids may be saturated or unsaturated or also semi-drying or drying fatty acids.

2. The emulsions contain a water-insoluble 35 water-proofing substance as dispersed constitu-

ent. Substances of this nature are paraffin, paraffin oil, mineral oil, vegetable oils and fats, resins, animal, vegetable or mineral waxes and latex, either singly or admixed.

3. A protective colloid which is soluble in water 5 and swells. Substances of this kind are glue, gelatine, starch, dextrin, vegetable slimes, casein, vegetable proteins, carrageon moss or the like.

4. The salt of a multivalent cation, which is added for the purpose of producing the soap of 10 the multivalent metal referred to under 1. This accordingly relates to the salt which is decomposed with the alkaline salt of the fatty acid according to 1. It is necessary to employ more salt than corresponds with the molecular conditions. 15 For example, to convert sodium soap into aluminum soap it is necessary to employ not the equivalent amount of aluminum salt, but an excess thereof. This feature was already included in the example given in the original papers filed 20 August 6, 1930. These features of the composition represent essential parts of the emulsions. Reference will also be made, however, to an additional feature which in numerous cases serves to enhance the properties of the emulsions. This 25 relates to

5. The addition of wetting agents of an organic kind, which cause the dispersed components to penetrate more readily into the threads or fabric. Wetting agents of this kind are alcohols, ketones, esters, organic bases or salts of the latter. By way of example reference may be made to the following representatives of these groups: ethyl alcohol, n-butanol, cyclohexanol, methyl-cyclohexanon, amyl acetate, pyridine 30 bases and triethanolamine formate. It is common to all of these wetting agents that in contradistinction to the usual substances of this kind they have no polar group which is capable of entering into a salt with the multivalent 35 cation.

The concentration of the emulsions does not constitute part of this invention. This may be adjusted as desired, dependent on the fact as to whether diluted emulsions are produced, which 40 are employed in immediate fashion for impregnation purposes, or whether there are produced concentrated emulsions, from which the impregnation liquor is obtained by dilution or dissolution. For reasons of economy, however, it is desirable to produce concentrated emulsions, for 45 example those in which the dispersal phase amounts to 10-30% or more of the emulsion.

An essential feature of the emulsions according 50 to the invention consists in the fact that 55

these are homogenized, i. e., that the aqueous dispersions or emulsions are forced in positive fashion through narrow slots, apertures or passages, in which connection there occurs a grinding action and in consequence a reduction in the size of the particles of the dispersed component. A machine, which is suitable for producing the emulsion in this fashion, together with its arrangement is described in detail by Otto Lange, in "Technik der Emulsionen", 1929 (Berlin), pages 77 to 80. The homogenization itself may take place at different temperatures and is dependent primarily on the viscosity of the product to be homogenized or on the melting point of the dispersed component. The higher the melting point of the oleaginous phase, the greater will be the homogenizing temperature which is required. The advantage of the homogenization is based on two factors. Owing to the small size of the particles the emulsions are extremely resistant to transport, frost and storage, whilst on the other hand solutions produced from the same are capable of resisting separation or creaming. These powers of resistance, however, do not interfere with the treatment of textile materials, and the small particles are picked up by the fibres and deposited and held in the interstices of the materials. This results in a uniform impregnating effect without deterioration of the finish or a dimming effect on the color. The emulsions produced in this way by homogenization reveal in the diluted state a Brownian movement of the molecules.

With regard to the production of the emulsions, it may be stated quite generally that the soaps of the multivalent metals, such as aluminum, are obtained by double decomposition, the aqueous solution of an alkali soap, in the presence of a protective colloid and in the presence of a water-proofing substance, being decomposed, whilst being stirred, with the aqueous solution of a salt of the multivalent metal. As a basis for the process there may be employed finished alkali soaps, or these may be formed during the process by the saponification of a fatty acid with alkali. There is utilised the emulsifying force of the forming or previously formed soap, and through the medium thereof there is emulsified the water-proofing component in water. The emulsions according to the invention also exhibit the phenomenon that owing to the presence of the salt which forms the multivalent soap, and more particularly, therefore, the aluminum salt, the dispersed component possesses a positive electrostatic charge, and in consequence is attracted by the textile fibres and is fixed thereon. This water-proof state produced in physical-chemical fashion is enhanced by the presence of the soap of the multivalent metal. This soap also assists towards proper adhesion of the impregnation substance.

As has been stated above, prior to the emulsification and homogenization, glue or other matter, which will swell when placed in water, is added to the alkali soap solution as an emulsifying medium, and I am able to use so much of the swelling matter, such as bone glue, that after mixing a semi-solid product may be obtained. I may also proceed in such a way that paraffin, wax and other water-proofing substances are homogenized with the aluminum soap emulsion, after so much of a swelling medium has been added as an emulsifying medium, that after cooling the emulsion, which preferably has been

homogenized at an elevated temperature, is solidified.

This solid product is able to emulsify with water, and it may be used in the same way as the products referred to above. 5

#### Examples

1. 14 kilograms of light pine-resin rosin are heated with 3.5 kilograms of table paraffin (melting point 52/54° C.) to 80-90° C. In 10 this there are then dissolved, whilst being stirred, 1.5 kilograms of 60% soap, which has been produced from palm-kernel oil and earth-nut oil by saponification with sodium lye. In a separate vessel 2 kilograms of gelatine in 15 pearl form are allowed to soak for 4 hours or longer in 5 kilograms of water, and by heating and stirring are then converted to a uniform solution. To this there are added 15.4 kilograms of water, both the gelatine solution as 20 well as the water having a temperature of 70° C., and the gelatine solution is then added under agitation to the above mixture of resin, paraffin and soap. An extremely finely distributed emulsion is obtained. In a third vessel 1.75 kilograms of 25 80% formic acid have been mixed with 6.65 kilograms of water, and in this mixture there have been dissolved 1.6 kilograms of hydrate of alumina, i. e., 50% aluminum hydroxide, which has been obtained by the precipitation of an aluminum salt with alkali, filtration and gentle drying. There is produced alumina formate, which at 18° C. possesses a spindle weight of 18° Bé.

The solution of aluminum formate thus obtained is added under agitation to the emulsion produced in the manner described above, and the latter, after being stirred for half an hour, when it has attained a completely uniform condition, is introduced into a three-pump homogenizing machine, such as described in the stated book by Lange, and is homogenized at 70-80° C. under a pressure of 120 atmospheres. This emulsion is allowed to cool either whilst being slowly and steadily stirred or without agitation 40 in a suitable metallic vessel. In the hot state the emulsion is a white viscous substance, and when cold solidifies to form a mass of gelatinous consistency which is capable of being cut. The product thus obtained is employed in the following manner:

In a metallic vessel 5 kilograms of the product obtained in the manner described are mixed under agitation with 8-10 kilograms of water having a temperature of 60° until a uniform and somewhat viscous solution of the emulsion has been formed. In the trough of a padding machine having a capacity of 100 litres there are heated 85 kilograms of water to 60° C., and the basic solution is then added 60 to the remainder of the water through a hairsieve. A wool-gabardine fabric is introduced in the dry condition into this liquor, squeezed out, dried, damped, pressed and cooled and finished off in the usual manner. This fabric has a 65 proper finish and possesses good water-repelling properties.

2. 110 parts paraffin (melting point 52/54° C.), 90 parts paraffin oil, 30 parts montan wax, and 6 parts soya fatty acid (an example of a semi-drying fatty acid) are emulsified under agitation with a solution of 2 parts potassium hydroxide (45° Bé.) and 240 parts water.

To this there are added 35 parts glue in 100 parts water, and into this solution there are 75

stirred 200 parts aluminum formate (17° Bé.), and after the emulsion has been evenly distributed it is homogenized at 150 atmospheres and at a temperature of 55° C. and then allowed to cool. This product is a white plastic substance.

In this example there will be described the use of wetting agents. If for this purpose there is employed an alcohol, it is incorporated in such fashion that it is added to the paraffin before, during or after the emulsifying in the soap solution. It is necessary that the wetting agent also be homogenized. When employing pyridine the procedure may be the same, or the pyridine may be added to the aqueous glue solution employed for emulsifying the fatty component. The ratio, for example, is 10 parts cyclohexanol or 6 parts pyridine to 1,000 parts emulsion.

3. 118.4 kilogrammes of table paraffin (melting point 52/54° C.), 64 kilogrammes of paraffin oil and 50 kilogrammes of the fatty acid of a semi-drying oil are melted together, and are emulsified in the hot state by pouring in 75 kilogrammes of an 8.2% potassium lye. Parallel thereto, after the dissolution of 15 kilogrammes of glue in 50 kilogrammes of water, this solution is mixed with the soap and paraffin emulsion. To enable the chemical decomposition to take place in satisfactory and reliable fashion glue is also added as a protective colloid to the aluminum salt or its aqueous solution, viz., in the following proportions: 28.2 kilogrammes of 80% formic acid are mixed with 212 kilogrammes of water, and in the same there are dissolved 24.8 kilogrammes of hydrate of alumina. To this solution there is added a solution of 20 kilogrammes of glue in 65 kilogrammes of water. The two reaction components, i. e., the aluminum formate solution and the emulsion of glue, soap and paraffin have a temperature of 60° C. The former is now added to the latter under agitation, and homogenization is likewise performed at 60° C. and at 150 atmospheres. After cooling the product is a white plastic mass. This product, as in Example 1, is dissolved, and a concentration of 20 grammes per litre at 50° C. is sufficient for impregnating a bleached cotton material in order to impart good water-repelling properties thereto.

4. In this example the composition is as follows: 133 parts Japanese wax, 53 parts vaseline, and the aluminum soap from 120 parts oil-soap and 200 parts alumina formate (17° Bé.).

The emulsification may take place, as in the above examples, by adding the part containing the aluminum salt to the fatty emulsion. Another method consists in presenting the fat in non-emulsified form in a melted condition, and then to stir into this melted phase the solution containing the aluminum salt and the aluminum soap, which solution also contains the protective colloid.

5. The operation as last described in conjunction with the proportions set forth in Example 2 takes the following form:

35 parts glue are dissolved in 100 parts of water, and in this solution there are emulsified 6 parts of a semi-drying fatty acid, for example rape-oil fatty acid. This is then converted to potassium soap by adding 2 parts potassium hydroxide (45° Bé.) and 240 parts water. To this solution of glue and soap there are added, under continuous agitation, 200 parts aluminum formate (17° Bé.) whereupon, by double decomposition between potassium soap on the one hand and the aluminum salt on the other hand, aluminum

soap is obtained, which remains emulsified in the solution of glue. This mixture is maintained between 55 and 60° C. In an agitating mechanism having a bladed stirrer performing approximately 300-400 R. P. M. there is placed a 5 melted mixture comprising 110 parts paraffin, 90 parts white oil and 30 parts montan wax. This mixture, which has a temperature of 60-70° C., is vigorously agitated, and the solution previously produced, as described above, is stirred 10 into the fatty substance. An emulsion is formed, which is thereupon homogenized at a pressure of 150 atmospheres. The product obtained is similar to that as set forth in Example 2. If desired, the homogenization may be repeated in 15 order still further to reduce the size of the particles. The product is also very suitable in greatly diluted solutions for water-proofing cotton goods or artificial silk and is remarkable for the fact that it in no way affects the finish of even 20 the finest artificial silk.

6. 40 parts table paraffin (52/54° C.), 40 parts paraffin oil and 10 parts ceresine (ozokerite) are admixed with 60 parts poppy oil fatty acid. 10 parts sodium hydroxide are dissolved in 150 parts 25 water, saponification being performed by stirring the fatty acid into the melted fatty substance, and in this way there is formed simultaneously, under agitation, an emulsion. The temperature amounts to 60° C. To this emulsion there is 30 added a solution comprising 55 parts glue in 350 parts water, likewise having a temperature of 60°, and copper soap is formed by adding to this solution whilst stirring 20 parts copper sulphate in 220 parts water. A slightly blue consistent emulsion is formed, which is thereupon homogenized at 60° C., and at 50° C. it is again passed through the machine under a pressure of 200 atmospheres. Cotton fabrics treated with a solution of this emulsion are waterproof and 35 also capable of resisting mildew and rusty stains.

The present application is a continuation in part of my co-pending application, Serial No. 555,148, filed August 4, 1931.

What I claim as new and desire to secure by 45 Letters Patent is:

1. Method of producing impregnating substances for water-proofing textile materials, which consists in emulsifying 110 parts paraffin (melting point 52-54° C.), 90 parts paraffin oil, 50 30 parts montan wax, 6 parts soya fatty acid and 10 parts cyclohexanol in a solution of 2 parts potassium hydroxide of 45° Bé., and 240 parts water, adding thereto a solution of 35 parts glue in 100 parts water, adding to the 55 whole 200 parts aluminum formate of 17° Bé., homogenizing the emulsion at 55° C. and at 150 atmospheres and thereupon allowing the emulsion to cool.

2. Method of producing impregnating substances for water-proofing textile materials, which consists in dissolving 35 parts glue in 100 parts water and emulsifying therein 6 parts rape-oil fatty acid, adding a solution comprising 2 parts potassium hydroxide of 45° Bé. and 240 60 parts water, stirring in 200 parts aluminum formate of 17° Bé., stirring the whole at a temperature of 60° C. into a melted mixture comprising 110 parts paraffin, 90 parts white oil and 30 parts montan wax and having a temperature 70 of 60-70° C., and thereupon homogenizing the emulsion produced at a pressure of 150 atmospheres.

3. A method of producing impregnating substances for water-proofing textile materials, 75

which consists in dissolving 35 parts glue in 100 parts water and emulsifying therein 6 parts of a semi-drying fatty acid and adding a solution containing 2 parts potassium hydroxide, water, and 200 parts of a formate of a metal selected from the group consisting of aluminum, magnesium, zinc, lead, and copper, adding thereto

110 parts paraffin, 90 parts paraffin oil, and 30 parts montan wax, and thereupon homogenizing the emulsion produced at a temperature of 55° to 70° centigrade and a pressure of at least 150 atmospheres.

RUDOLF KERN.